

## UNITED STATES PATENT OFFICE

2,185,905

PROCESS FOR THE PRODUCTION OF FAST  
TINTS ON VEGETABLE FIBERSFritz Straub, Basel, Walter Hanhart, Riehen, near  
Basel, and Walter Anderau, Basel, Switzerland,  
assignors to the firm of Society of Chemical  
Industry in Basle, Basel, SwitzerlandNo Drawing. Application December 15, 1936, Se-  
rial No. 116,038. In Switzerland December 19,  
1935

8 Claims. (Cl. 8—42)

It has been found that fast tints can be obtained on vegetable fibers, for instance cotton, if dyeings of complex metal compounds of direct cotton dyestuffs are produced on vegetable fibers, at least one phase of the process being carried out in a caustic alkaline medium at a raised temperature.

By direct cotton dyestuffs are to be understood those di- and polyazo-dyestuffs which have affinity for vegetable fibers. Such dyestuffs may be constructed from diazotized aromatic amines which impart to the dyestuffs an affinity for vegetable fiber for instance cotton and artificial silk from regenerated cellulose, and from any coupling components, for instance phenols, naphthols or amines of the benzene and naphthalene series; or such dyestuffs may be made by coupling any diazotized aromatic amine with a coupling component which imparts to the dyestuff an affinity for vegetable fiber. There may also be used direct cotton dyestuffs derived from diazo-components which impart to the dyestuffs affinity for vegetable fiber, and also coupling components having the same property. The components for the manufacture of the direct cotton dyestuffs are selected in such a manner that the dyestuff contains at least one lake-forming group; such components are, for example, the diazo-compounds which contain in ortho-position to the diazo-group or in ortho-position or peri-position to a cyclic tertiary nitrogen atom a hydroxyl-, a carboxyl- or an alkoxy-group or a salicylic acid grouping, or coupling components which contain the salicylic acid grouping as a substituent.

In the foregoing statement it will be seen that for the construction of the direct cotton dyestuffs there come into consideration not only the usual aromatic amines of the benzene and naphthalene series which contain lake-forming groups for the purpose of diazo-components and not only the usual phenols, naphthols and amines for the purpose of coupling components but also, in particular, direct-dyeing components, such as, for example, benzidine or stilbene derivatives, diaryl-azoxy-derivatives and carbazole derivatives, urea and thiourea from arylendiamines, acetoacetic acid derivatives, pyrazolones, aminonaphthols and their sulfonic acids.

The process is of particular value for direct dyeing dyestuffs containing lake-forming groups, the complex metallic compounds of which are sparingly soluble to insoluble in water; to these dyestuffs belong those which contain only few or no groups lending solubility, for instance sulfo-

groups or carboxyl-groups, or which contain such groups lending solubility as, for example, the salicylic acid group, if desired in addition to the sulfo-groups, which groups combine with metal and thereby lose entirely or partly their power of lending solubility.

The production of complex metal compounds of direct cotton dyestuffs on vegetable fibers according to the present process may be effected in such a manner that the fibers are dyed with direct cotton dyestuffs containing groups capable of forming lakes, and the dyeings thus obtained treated with agents yielding metal, the operation being conducted in at least one phase of the process in a hot caustic alkaline medium.

The operation of dyeing vegetable fibers with dyestuffs according to this invention may follow the lines usual in applying direct cotton dyestuffs, that is to say the dyeing may be conducted in a bath containing Glauber's salt, preferably also alkali carbonate, for instance sodium carbonate, or the goods may be dyed at a raised temperature in a medium containing caustic alkali, for instance caustic soda or caustic potash. In many cases, particularly in those in which the dyestuff used affords complex metal compounds which are sparingly soluble to insoluble in water, it is of advantage to bring the dyestuff, before dyeing, for example by grinding, into a fine state of subdivision or/and to dye in presence of a dispersing, wetting or emulsifying agent, that is to say in the presence of anion or cation capillary active substances or such capillary active substances which are not ionised. Such substances are, for example, organic derivatives of ammonia, for instance amines of the aliphatic, hydroaromatic and aromatic series, which may contain hydroxyl-groups or other substituents, (for example pyridine, amines, alkylamines, ethanolamine, cyclohexylethanolamine, butylethanolamine), sulfonic acids of the benzene and naphthalene series which contain alkyl-groups, alcohols, for instance glycerine; also alcohol sulfonates, soluble condensation products of fatty acids of high molecular weight or of ethylene oxide and amines; oxyoleic acids, sulforicinates, glue, sulfite cellulose liquor, dextrin, albuminous degradation products, for instance protalbinic acid or lysalbinic acid, or organic compounds of high molecular weight, such as the polymerisation products of aldehydes and soluble degradation products of cellulose. In case the dyeing is performed with the dyestuffs containing the lake-forming groups by the usual methods, for example in the presence of Glauber's salt, and if desired also alkali

5

10

15

20

25

30

35

40

45

50

55

carbonate, the after-treatment of the dyeing with the agent which yields the metal in complex union, may occur in the same bath or in a fresh bath, in presence of the necessary caustic 5 alkaline medium and at a raised temperature.

When the dyeing with the dyestuff containing the lake-forming group occurs in a caustic alkaline medium at a raised temperature the after-treatment with the agent yielding the complex 10 bound metal, which may happen in the same or in a fresh bath, may be carried out either by one of the usual methods, for instance by treating the dyeing, if necessary after neutralizing the dye-bath in a neutral or acid medium, with the usual 15 agents that yield metal, such as chromium, cobalt, nickel, manganese, aluminium, zinc, vanadium, titanium, and, in particular, copper, or this after-treatment may be applied simultaneously 20 with the dyeing in the caustic alkaline medium at the raised temperature. In this caustic alkaline 25 after-treatment at the raised temperature, which may occur in presence of the aforesaid dispersing, wetting or emulsifying agent, there are preferably used such agents yielding complex bound 30 metal which are stable to dilute caustic alkalies and correspondingly are only feebly hydrolysed in a caustic alkaline medium or not hydrolysed at all. Such agents are, for example, the aqueous 35 solutions having alkaline reaction which are obtained by mixing the product of the action of an ordinary agent, yielding metal which may contain several metals on an aliphatic hydroxycarboxylic acid (for example lactic acid, tartaric acid, glycolic acid, tartaric acid, malic acid, di- 40 oxytartaric acid, citric acid, saccharic acid, gluconic acid or heptonic acid) or on an amino-carboxylic acid (for example glycocoll) with, for instance, caustic soda solution, caustic potash solution, ammonia, or a derivative of ammonia, for example ethanolamine, until alkaline reaction is 45 produced.

The production of complex metal compounds of direct cotton dyestuffs on vegetable fibers according to the present process may also be effected in such a manner that the fiber is dyed at a raised temperature with complex metal compounds of direct cotton dyestuffs in a caustic alkaline medium containing, for example, caustic soda or caustic potash lye. These complex metal 45 compounds can be made, with or without the application of pressure, from the aforesaid direct cotton dyestuffs containing lake-forming groups in the usual manner, for instance by treatment with an agent yielding chromium, cobalt, nickel, aluminium, manganese, zinc, vanadium, titanium and, in particular, copper, in presence or absence of the usual additions, for example an inorganic salt or acid or an organic salt or acid, with or without application of pressure. Particularly 50 good results are obtained when sparingly soluble to insoluble complex metal compounds are used which may be made in the dye-bath. It is advantageous in many cases that these dyestuffs should be reduced to a finely divided state, that is to say to a highly dispersed form before the dyeing, which is possible, for example, by grinding the dyestuff in the form of a powder or containing a liquid medium, for example in the form of an aqueous paste, in the usual apparatus, such 55 as a ball-mill or a roller mill, or by wind sifting; or if in the metallizing operation there is present, for example an aliphatic hydroxycarboxylic acid or a derivative of ammonia, for instance ethanolamine, or an amino-carboxylic acid, for 60 instance amino-acetic acid; for in such cases the 65 70 75

complex metal compound insoluble in water may pass into solution. These solutions may then be added to the dye-bath, in case the metallizing has not been already carried out in the dye-bath. There may also be added to the dye-bath, together with the agent yielding metal, such an amine or hydroxycarboxylic acid and a complex metal compound or a mixture of this amine or hydroxycarboxylic acid with the complex metal compound obtainable by, for instance, grinding the amine or hydroxycarboxylic acid with the dyestuff. As in the case of dyeing with direct cotton dyestuffs containing lake-forming groups, it is also in many cases advantageous, when using the complex metal compounds of the direct cotton dyestuffs, to dye in presence of the aforesaid dispersing, wetting or emulsifying agents.

The dyeings obtained by the process of the invention may be developed by treatment, if desired, in a fresh bath for some time with soap or 20 soap and sodium carbonate at about 50-75° C.

The dyeings obtained are strong colors and are distinguished by advantageous tints as well as by good fastness, for instance to washing and to light.

The following examples illustrate the invention, the parts being by weight unless otherwise stated and the relationship of parts by weight to parts by volume being that of the kilo to the litre:

#### Example 1

0.075 part of the azo-dyestuff of the formula



obtainable by coupling 1 mol. tetrazotized 4:4'-diaminostilbene-3:3'-dicarboxylic acid, on the one hand with 1 mol. phenyl-2-naphthylamine and on the other hand with 1 mol. 5:5'-dihydroxy-2:2'-dinaphthylamine-7:7'-disulfonic acid, is dissolved in 200 parts of water. There are added 1.2 parts by volume of caustic soda solution of 30 per cent. strength and 3 parts of Glauber's salt, and 10 parts of cotton are entered at 30-40° C. The bath is heated to boiling and dyeing is continued at this temperature for 45 minutes. There are then added to the same bath 20 parts of a caustic alkaline copper solution made by dissolving together 10 parts of crystallized copper sulfate, 12 parts of tartaric acid and 15 parts of caustic soda in 1000 parts of water. The goods are handled for about 30 minutes at 90-100° C. and then thoroughly rinsed with cold water.

The dyeing obtained is of a considerably purer blue as well as stronger and more level than the dyeing produced from the same dyestuff by the usual after-treatment with a copper compound.

Similar results can be obtained if instead of tartaric acid there is used an equivalent proportion of saccharic acid.

The after-treatment with copper may be conducted also at a lower temperature; indeed, in the cold.

**Example 2**

0.05 part of the dyestuff of the formula



from 1 mol. tetrazotized 4:4'-diaminodiphenyl and 2 mols. 6-methyl-1-hydroxy-benzene-2-carboxylic acid is dissolved in 200 parts of water containing 1.2 parts by volume of caustic soda solution of 30 per cent. strength. To this bath there are added 3 parts of Glauber's salt and 10 parts of cotton are entered at 30-40° C. The bath is heated to boiling and dyeing continued for 45 minutes at 95-100° C. There are then added 20 parts of caustic alkaline solution of copper, made by dissolving 10 parts of crystallized copper sulfate, 12 parts of tartaric acid and 15 parts of caustic soda in 1 litre of water. The goods are handled for about 30 minutes at 90-100° C. and then thoroughly rinsed in cold water.

The dyeing obtained is of better fastness to washing and stronger than that obtained with use of the same dyestuff by the usual after-treatment with copper.

Similar results can be obtained if instead of tartaric acid there is used an equivalent proportion of glycollic acid.

A like result is obtained if the caustic alkaline copper solution is added to the dye-bath in the first instance.

The proportion of caustic alkali necessary in the dye-bath may vary within wide limits.

**Example 3**

45 The dye-bath is prepared from 200 parts of water at 30-40° C., 0.3 part of Glauber's salt and 0.1 part of the copper compound of the formula



65 obtainable in the known manner from 1 mol. tetrazotized 4:4'-diamino-diphenyl-3:3'-dicarboxylic acid and 1 mol. each of phenyl-2-naphthylamine and 1-amino-8-hydroxynaphthalene-4-sulfonic acid and made into the form of a

paste with 1.6 parts of caustic soda solution of 30 per cent. strength 0.3 part of tartaric acid and 10 parts of water, and warming for a short time to produce a solution. 10 parts of cotton are then entered, the bath is heated to boiling in the course of half-an-hour and this temperature is maintained for about 1 hour. The goods are then washed thoroughly with cold water. Reddish blue tints of good fastness to washing are obtained.

Similar results can be obtained if instead of tartaric acid there is used an equivalent proportion of glycollic acid amide.

**Example 4**

A dye-bath is prepared from 200 parts of water, at 30-40° C. 0.3 part of Glauber's salt and 0.1 part of the copper compound obtained in known manner from the dyestuff from 1 mol. tetrazotized 4:4'-diamino-diphenyl-3:3'-dicarboxylic acid and 1 mol. each of phenyl-2-naphthylamine and 1-amino-8-hydroxynaphthalene-4-sulfonic acid, which is first made into the form of a paste by means of 3.2 parts of caustic soda solution of 30 per cent. strength, 0.6 part of tartaric acid and 0.125 part of crystallised copper sulfate, as well as 15 parts of water, and then heating for a short time until dissolution occurs. 10 parts of cotton are now entered, the bath is heated to boiling in the course of half-an-hour, and kept at this temperature for about 1 hour. Thorough rinsing with cold water follows. There is obtained a blue dyeing of good fastness to washing.

Similar results can be obtained if instead of tartaric acid there is used an equivalent proportion of malonic acid mono-amide.

**Example 5**

40 Into a dye-bath consisting of 1500 parts of water, 1 part of caustic soda solution of 36° Bé., 30 parts of Glauber's salt and 1 part of glycerine, as well as 1 part of the dyestuff described in Example 9, first paragraph of Specification No. 1,861,323, 100 parts of cotton are entered at 30-40° C. The bath is heated in the course of half-an-hour to 90-100° C. and this temperature is maintained for another quarter of an hour and there is added a solution made by mixing a solution of 0.5 part of copper sulfate and 0.5 part of tartaric acid in 2 parts of water with caustic soda solution until the reaction is feebly alkaline. Dyeing is continued for 15-20 minutes at about 90° C. and the goods are then rinsed and dried. Before drying it may be advantageous to apply a fresh bath at 50° C. containing per litre 0.5 part of Marseilles soap so as to soap the dyeing for 1/2 hour. A very good orange tint fast to light and washing is obtained.

55 Similar results can be obtained if instead of tartaric acid there is used an equivalent proportion of ammonium citrate.

**Example 6**

60 Into a dye-bath containing 1500 parts of water, 1 part of caustic soda solution of 36° Bé., 30 parts of Glauber's salt and 0.5 part of cane or beet sugar, as well as 1 part of the dyestuff of the formula



there are entered at 30-40° C., 100 parts of cotton. The temperature is raised in the course of half-an-hour to 90-100° C. and dyeing is continued for half-an-hour at the same temperature.

- 5 There is now added to the dye-bath a solution made by mixing a solution of 0.5 part of copper sulfate and 0.5 part of tartaric acid in 2-3 parts of water with caustic soda solution until the reaction is feebly alkaline with caustic alkali.
- 10 Dyeing is further continued for 15-20 minutes, whereupon the goods are rinsed and soaped in a soap bath of 1/2 per cent. strength and at 50° C. and then rinsed and dried. A blue tint of very good fastness to light and washing is obtained.

15 Instead of 0.5 part of sugar there may be used 1-2 parts of ethyl alcohol and instead of tartaric acid an equivalent proportion of lactic acid.

If in this example there is substituted for the



dyestuff indicated the tetrakisazo-dyestuff of the formula



a reddish blue fast to light and washing is obtained.

*Example 7*

- 40 Into a dye-bath consisting of 700 parts of water, 0.2 part of the dyestuff of the formula



- 50 2 parts of caustic soda solution of 36° Bé., 6 parts of crystallized Glauber's salt and a solution made from 10 parts of water, 0.25 part of crystallized copper sulfate, 0.55 part of potassium sodium tartrate and 3 parts of a caustic soda solution of 40 per cent. strength are entered at 40° C., 20 parts of cotton. In the course of half-an-hour the bath is heated to boiling and kept at this temperature for about three-quarters of an hour to 1 hour. The goods are then thoroughly rinsed with cold water and soaped in a fresh bath at 50° C. with 5 grams of Marseilles soap per litre of liquor for about half-an-hour.

55 There is obtained a blue dyeing which is purer, more level, faster to washing and stronger than that obtained by the dyeings produced by the known processes.

60 Similar results can be obtained if instead of potassium sodium tartrate there is used an equivalent proportion of amino-tartaric acid.

*Example 8*

- 65 Into a dye-bath consisting of 1500 parts of water, 1 part of the dyestuff used in Example 9, first paragraph of Specification No. 1,861,323 and 2 parts of calcined sodium carbonate, 100 parts of cotton are entered at 30-40° C. The

5 dye-bath is heated to boiling in the course of half-an-hour and there are added 30 parts of Glauber's salt, dyeing being continued for about 3/4 hour at the said temperature. There is then added to the bath a solution made by mixing an aqueous solution of 0.4 part of chromium sulfate, 0.3 part of nickel sulfate and 0.6 part of tartaric acid with dilute caustic soda solution until the reaction is alkaline and the dyeing is continued for 30 minutes at 90-100° C. Rinsing and drying follow. Orange dyeings are obtained which have good fastness to washing and light.

10 Similar results can be obtained if instead of tartaric acid there is used an equivalent proportion of tartronic acid.

*Example 9*

15 100 parts of cotton are dyed with 1 part of the dyestuff of the formula

20 in 1500 parts of water in presence of 2 parts of calcined sodium carbonate and 30 parts of Glauber's salt, the dyeing being continued for 3/4 hour at 90-100° C. There is then added a solution obtained by mixing a solution of 0.1 part of cobalt hydroxide in 1 part of ammonia of 24 per cent. strength with a caustic alkali solution of

25 30 35

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5

action is caustic alkaline. Dyeing is continued further for 30 minutes at 90-100° C. and the goods are rinsed and dried. Fast yellow tints are obtained, the fastness to washing of which may be subsequently improved by treatment in a soap bath or a soda-soap bath.

Similar results can be obtained if instead of tartaric acid there is used an equivalent proportion of malic acid.

10 *Example 11*

Into a dye-bath consisting of 700 parts of water, 0.2 part of the dyestuff of the formula:



- thylamine-7:7'-disulfonic acid, 10 parts of cotton are entered, the bath is heated to boiling in the course of half-an-hour and kept at this temperature for about 45 minutes. There are then added to the dye-bath 0.2 part of the sodium salt of the sulfonated condensation product from benzyl chloride and naphthalene and 20 parts of a caustic alkaline copper solution containing in 1000 parts by volume 10 parts of crystallized copper sulfate, 12 parts of tartaric acid and 15 parts of caustic soda. Dyeing is continued for about 30 minutes at 95-100° C. and the material is then rinsed with cold water, soaped if necessary and dried. There is obtained a fast blue dyeing.
- Similar results can be obtained if instead of tartaric acid there is used an equivalent quantity of glycollic acid, or if instead of the sodium salt of the sulfonated condensation product from benzyl chloride and naphthalene there is used 0.2 part of the sodium salt of sulfophthalic acid diamyl ester.

*Example 16*

- A dye-bath is prepared from 200 parts of water at 30-40° C., 3 parts of Glauber's salt and 0.1 part of the azo-dyestuff obtained by coupling 1 mol. of tetrazotized 4:4'-diaminodiphenyl-3:3'-dicarboxylic acid with 1 mol. each of 2-phenylaminonaphthalene and 1-amino-8-hydroxynaphthalene-4-sulfonic acid, 10 parts of cotton are entered, the bath is heated to boiling in the course of half-an-hour and dyeing is continued for 45 minutes at this temperature. There are then added to the dye-bath 20 parts of an alkaline copper solution containing in 1000 parts by volume 10 parts of crystallized copper sulfate, 12 parts of tartaric acid and 15 parts of caustic soda. Dyeing is continued for about 30 minutes at 95-100° C. and the material is then thoroughly rinsed with cold water, soaped in known manner and dried. There is obtained a reddish-blue dyeing which is faster to alkali than one produced by the usual process of after-treatment with copper.

- Similar results can be obtained if instead of tartaric acid there is used an equivalent quantity of glycollic acid or/and if instead of copper sulfate there is used an equivalent quantity of nickel sulfate.

*Example 17*

- A dye-bath is prepared from 200 parts of water at 30-40° C., 3 parts of Glauber's salt and 0.25 part of a paste of 35 per cent. strength of the azo-dyestuff of the formula



carboxylic acid and 1-(4'-hydroxy-3'-carboxy)-phenyl-3-methyl-5-pyrazolone, 10 parts of cotton are entered, the bath is heated to boiling in the course of half-an-hour and dyeing is continued for 45 minutes at this temperature. There are then added to the dye-bath 20 parts of an alkaline copper solution containing in 1000 parts by volume 10 parts of crystallized copper sulfate, 12 parts of tartaric acid and 15 parts of caustic soda. Dyeing is continued for about 30 minutes longer at 95-100° C., and the goods are thoroughly rinsed with cold water and dried. There is obtained a very fast red-brown dyeing.

Similar results can be obtained if there is used instead of tartaric acid an equivalent quantity of aminotartaric acid and/or instead of copper sulfate an equivalent quantity of nickel sulfate.

*Example 18*

A dye-bath is prepared from 200 parts of 20 water at 30-40° C., 3 parts of Glauber's salt and 0.25 part of a paste of 35 per cent. strength of the azo-dyestuff from tetrazotized 4:4'-diaminodiphenyl-3:3'-dicarboxylic acid and 1-(4'-hydroxy-3'-carboxy)-phenyl-3-methyl-5-pyrazolone, 10 parts of cotton are entered, the bath is heated to boiling in the course of half-an-hour and dyeing is continued for 45 minutes at this temperature. There are then added to the dye-bath 20 parts of an alkaline copper solution containing in 1000 parts by volume 10 parts of crystallized copper sulfate, 12 parts of tartaric acid, 15 parts of caustic soda and 10 parts of a solution of ammonia of 24 per cent. strength. Dyeing is continued for about 30 minutes longer at 95-100° C., and the goods are thoroughly rinsed with cold water and dried. There is obtained a very fast red-brown dyeing.

Similar results can be obtained if there is used instead of tartaric acid an equivalent quantity of glycollic acid and/or instead of copper sulfate an equivalent quantity of nickel sulfate.

*Example 19*

A dye-bath is prepared from 200 parts of 45 water at 30-40° C., 3 parts of Glauber's salt and 0.25 part of a paste of 35 per cent. strength of the azo-dyestuff from tetrazotized 4:4'-diaminodiphenyl-3:3'-dicarboxylic acid and 1-(4'-hydroxy-3'-carboxy)-phenyl-3-methyl-5-pyrazolone, 10 parts of cotton are entered, the bath is heated to boiling in the course of half-an-hour and dyeing is continued for 45 minutes at this temperature. There are then added to the dye-bath 0.2 part of an emulsifying agent prepared 55 from glue and soap and 20 parts of an alkaline copper solution containing in 1000 parts by volume 10 parts of crystallized copper sulfate, 12 parts of tartaric acid and 15 parts of caustic soda. Dyeing is continued for about 30 minutes longer at 95-100° C. and the material is then thoroughly rinsed with cold water, if necessary soaped in the usual manner and dried. There is obtained a fast red-brown dyeing which alters less when washed than a dyeing which 60 has been after-coppered according to known processes.

Similar results can be obtained if there is used instead of tartaric acid an equivalent quantity of glycollic acid and/or instead of copper sulfate an equivalent quantity of nickel sulfate.

*Example 20*

For dyeing 100 parts of cotton-satin a dye-bath of temperature 50° C. is prepared from 75

4000 parts of water and 2.5 parts of the copper compound of the dyestuff of the formula



of  $\frac{1}{4}$  hour the temperature is raised to  $95^{\circ}$  C.; 30 parts of crystallized Glauber's salt are now added and dyeing is continued for 30 minutes longer at  $95^{\circ}$  C. There is then added to the dye-bath an alkaline solution prepared by mixing aqueous solutions of 1.5 parts of crystallized copper sulfate, 1.2 parts of potassium tartrate and 0.6 part of caustic soda. Dyeing is continued for 30 minutes longer at  $90-95^{\circ}$  C. and the material is then rinsed with cold water. There is obtained a powerful orange dyeing which is fast to light and to washing. The dyeing is brighter, considerably stronger and of better fastness to alkali than one which has been after-treated with copper sulfate in a fresh bath according to known methods.

Similar results are obtained if instead of tar-  
taric acid an equivalent quantity of saccharic  
acid is used.

20

*Example 22*

For dyeing 100 parts of cotton-satin a dye-bath of temperature  $50^{\circ}$  C. is prepared from 4000 parts of water and 2.5 parts of the dyestuff of the formula

25



the wetted cotton is introduced and in the course of  $\frac{1}{4}$  hour the temperature is raised to  $95^{\circ}$  C.; 30 parts of crystallized Glauber's salt are now added and dyeing is continued for 30 minutes longer at  $95^{\circ}$  C. There is then added to the dye-bath an alkaline solution prepared by mixing aqueous solutions of 1.5 parts of crystallized copper sulfate, 1.2 parts of potassium tartrate and 0.6 part of caustic soda. Dyeing is continued for 30 minutes longer at  $90-95^{\circ}$  C. and the material is then rinsed with cold water. There is obtained a powerful brown dyeing which is fast to light and to washing. The dyeing is brighter, considerably stronger and of better fastness to alkali than one which has been after-treated with copper sulfate in a fresh bath according to known methods.

Similar results are obtained if instead of potassium tartrate an equivalent quantity of glycollic acid amide is used.

*Example 21*

For dyeing 100 parts of cotton-satin a dye-bath of temperature  $50^{\circ}$  C. is prepared from 4000 parts of water and 2.5 parts of the dyestuff of the formula



the wetted cotton is introduced and in the course of  $\frac{1}{4}$  hour the temperature is raised to  $95^{\circ}$  C.; 30 parts of crystallized Glauber's salt are now added and dyeing is continued for 30 minutes longer at  $95^{\circ}$  C. There is then added to the dye-bath an alkaline solution prepared by mixing aqueous solutions of 1.5 parts of crystallized copper sulfate, 1.2 parts of potassium tartrate and 0.6 part of caustic soda. Dyeing is continued for 30 minutes longer at  $90-95^{\circ}$  C. and the material is then rinsed with cold water. There is obtained a powerful yellow dyeing which is fast to light and to washing. The dyeing is considerably stronger and of better fastness to alkali than one which has been after-treated with copper sulfate in a fresh bath according to known methods.

Similar results are obtained if instead of copper sulfate an equivalent quantity of nickel sulfate is used; instead of potassium tartrate there may be used an equivalent quantity of sodium saccharate.

60

50

55

*Example 23*

For dyeing 100 parts of cotton-satin a dye-bath of temperature  $50^{\circ}$  C. is prepared from 4000 parts of water and 2.5 parts of the dyestuff of the formula

65

the wetted cotton is introduced and in the course



the wetted cotton is entered and the temperature is raised in the course of  $\frac{1}{4}$  hour to 95° C.; 30 parts of crystallized Glauber's salt are added and dyeing is continued for 30 minutes longer at 95° C. There is then added to the dye-bath an alkaline solution prepared by dissolving in water 1.5 parts of crystallized copper sulfate, 1.2 parts of potassium tartrate and 0.6 part of caustic soda. Dyeing is continued for 30 minutes longer at 90-95° C. and the material is then rinsed with cold water. There is obtained a powerful yellow dyeing which is fast to light and to washing. It is considerably stronger and of better fastness to alkali than a dyeing obtained by after-treatment 15 with copper sulfate in a fresh bath according to known processes.

Similar results are obtained if instead of copper sulfate an equivalent quantity of nickel sulfate is used, and if instead of potassium tartrate 20 an equivalent quantity of sodium glycolate is used.

#### Example 24

0.075 part of the azo-dyestuff obtained by coupling 1 mol. of tetrazotized 4:4'-diamino 25 stilbene-3:3'-dicarboxylic acid on the one side with 1 mol. of phenyl-2-naphthylamine and on the other side with 1 mol. of 5:5'-dihydroxy-2:2'-dinaphthylamine-7:7'-disulfonic acid, is dissolved in 200 parts of water. 1.2 parts by volume 30 of caustic soda solution of 30 per cent. strength and 3 parts of Glauber's salt are added and 10 parts of cotton are entered at 30-40° C. The temperature of the bath is raised to boiling and dyeing is continued for 45 minutes at this temperature. The bath is then neutralized by addition of 0.86 part by volume of acetic acid of 84 per cent. strength, 0.2 part of crystallized copper 35 sulfate is added in the form of an aqueous solution and the goods are handled in the bath for about 30 minutes at 90-100° C., rinsed and dried. There is obtained a blue dyeing of good properties of fastness.

Similar results can be obtained by using instead of 0.2 part of crystallized copper sulfate an equivalent quantity of neutral sodium copper tartrate.

#### Example 25

0.075 part of the azo-dyestuff obtained by coupling 1 mol. of tetrazotized 4:4'-diamino 50 stilbene-3:3'-dicarboxylic acid on the one side with 1 mol. of phenyl-2-naphthylamine and on the other side with 1 mol. of 5:5'-dihydroxy-2:2'-dinaphthylamine-7:7'-disulfonic acid, is dissolved in 200 parts of water. 1.2 parts by volume 55 of caustic soda solution of 30 per cent. strength and 3 parts of Glauber's salt are added and 10 parts of cotton are entered at 30-40° C. The temperature of the bath is raised to boiling and dyeing is continued for 45 minutes at this temperature. The bath is then neutralized by addition of 0.86 60 part by volume of acetic acid of 84 per cent. strength, 0.2 part of crystallized nickel sulfate is added in the form of an aqueous solution and the goods are handled in the bath for about 30 minutes at 90-100° C., rinsed and dried. There is obtained a blue-violet dyeing of good properties of fastness.

#### Example 26

0.075 part of the azo-dyestuff obtained by coupling 1 mol. of tetrazotized 4:4'-diaminostilbene-3:3'-dicarboxylic acid on the one side with 1 mol. of phenyl-2-naphthylamine and on the other side with 1 mol. of 5:5'-dihydroxy-2:2'-dinaphthylamine-7:7'-disulphonic acid, is dissolved in

200 parts of water. 1.2 parts by volume of caustic soda solution of 30 per cent. strength and 3 parts of Glauber's salt are added and 10 parts of cotton are entered at 30-40° C. The temperature of the bath is raised to boiling and dyeing is continued for 45 minutes at this temperature. Then there are added to the same bath 20 parts of a caustic alkaline copper solution obtained by dissolving 10 parts of crystallized copper sulfate, 6.08 parts of glycolic acid and 15 parts of caustic soda in 10. 1000 parts of water. The goods are thoroughly rinsed with cold water. There is obtained a blue dyeing of good properties of fastness.

Similar results are obtained by using tartaric acid amide instead of glycolic acid.

#### Example 27

A dye-bath is prepared from 200 parts of water at 30-40° C., 0.6 part by volume of caustic soda solution of 30 per cent. strength, 3 parts of crystallized Glauber's salt and 0.8 part of the copper compound of the azo-dyestuff used in Example 22, 10 parts of cotton are entered, the bath is raised to boiling in the course of half-an-hour and dyeing is continued for about  $\frac{3}{4}$  hour at 25. 90-100° C. The goods are then thoroughly rinsed with cold water and dried. There is obtained a fast yellow dyeing.

Similar results can be obtained by using the nickel compound of the dyestuff instead of the copper compound.

#### Example 28

A dye-bath is prepared from 200 parts of water at 30-40° C., 0.6 part by volume of caustic soda solution of 30 per cent. strength, 3 parts of crystallized Glauber's salt and 0.8 part of the copper compound of the azo-dyestuff used in Example 22 as well as 0.5 part of protalbinic acid, 10 parts of cotton are entered, the bath is raised to boiling in the course of half-an-hour and dyeing is continued for about  $\frac{3}{4}$  hour at 90-100° C. The goods are then thoroughly rinsed with cold water and dried. There is obtained a fast yellow dyeing.

Similar results can be obtained if instead of protalbinic acid an equivalent quantity of lysalbinic acid is used.

#### Example 29

A dye-bath is prepared from 200 parts of water at 30-40° C., 0.6 part by volume of caustic soda solution of 30 per cent. strength, 3 parts of crystallized Glauber's salt and 0.8 part of the copper compound of the azo-dyestuff used in Example 23, 10 parts of cotton are entered, the bath is raised to boiling in the course of half-an-hour and dyeing is continued for about  $\frac{3}{4}$  hour at 90-100° C. The goods are then thoroughly rinsed with cold water and dried. There is obtained a fast yellow dyeing.

Similar results can be obtained by using a copper-chromium compound of the dyestuff instead of the copper compound.

#### Example 30

A dye-bath is prepared from 200 parts of water at 30-40° C., 0.6 part by volume of caustic soda solution of 30 per cent. strength, 3 parts of crystallized Glauber's salt and 0.8 part of the copper compound of the azo-dyestuff used in Example 23, as well as 0.5 part of an oxyoleic acid such as Monopole soap, 10 parts of cotton are entered, the bath is raised to boiling in the course of half-an-hour and dyeing is continued for about  $\frac{3}{4}$  75

hour at 90-100° C. The goods are then thoroughly rinsed with cold water and dried. There is obtained a fast yellow dyeing.

5 Similar results can be obtained by using a sulfo-ricinate instead of the Monopole soap.

*Example 31*

A dye-bath is prepared from 400 parts of water at 30-40° C. and 0.25 part of the chromium-copper compound prepared in known manner 10 from the dyestuff of the formula.



25 10 parts of cotton are entered and the temperature is raised to 95° C. in the course of 1/4 hour; then 3 parts of crystallized Glauber's salt are added and dyeing is continued for 30 minutes longer at 95° C. There is then added to the same dye-bath a caustic alkaline solution prepared by dissolving in water 1.5 parts of crystallized copper sulfate, 1.2 parts of potassium tartrate and 0.6 parts of caustic soda. Dyeing is continued for 30 minutes longer at 90-95° C. and the goods are then rinsed with cold water and dried. There is obtained a grey dyeing fast to light and to washing. It is brighter, has a more greenish hue and is faster to washing than a dyeing obtained by dyeing the material directly 30 with the same chromium-copper compound; it is also faster to washing than a dyeing obtained by after-treating the same chromium-copper compound with copper sulfate in a fresh bath by the usual processes.

40 *Example 32*

A dye-bath is prepared from 400 parts of water at 30-40° C. and 0.25 part of the chromium compound prepared in known manner from the azo-dyestuff referred to in Example 31, 10 parts of cotton are entered and the temperature is raised to 95° C. in the course of 1/4 hour; then 3 parts of crystallized Glauber's salt are added and dyeing is continued for 30 minutes longer at 95° C. 45 There is then added to the same dye-bath a caustic alkaline solution prepared by dissolving in water 1.5 parts of crystallized copper sulfate, 1.2 parts of potassium tartrate and 0.6 part of caustic soda. Dyeing is continued for 30 minutes longer 50 at 90-95° C. and the goods are then rinsed with cold water and dried. There is obtained a grey dyeing fast to light and to washing. It has a more greenish hue and is faster to washing than a dyeing obtained by dyeing the material directly 55 with the same chromium compound; it is also faster to washing than a dyeing obtained by after-treating the azo-dyestuff with copper sulfate in a fresh bath by the usual processes.

60 What we claim is:

65 1. Process for the production of fast tints on vegetable fibers, comprising producing dyeings of complex metal compounds of direct cotton dyestuffs on vegetable fibers, wherein at least once in the course of the dyeing process the vegetable fibers are treated in a caustic alkaline medium

at a raised temperature not exceeding the boiling point of the said medium.

2. Process for the production of fast tints on vegetable fibers, comprising dyeing the fibers with direct cotton dyestuffs containing lake-forming groups, and treating the dyeings with agents yielding metal, wherein at least once in the course of the dyeing process the vegetable fibers are treated in a caustic alkaline medium at a raised temperature not exceeding the boiling point of the said medium.

3. Process for the production of fast tints on vegetable fibers, comprising dyeing the fibers with complex metal compounds of direct cotton dyestuffs in a caustic alkaline medium at a raised temperature not exceeding the boiling point of the said medium.

4. Process for the production of fast tints on vegetable fibers, comprising dyeing the fibers with direct cotton dyestuffs containing lake-forming groups, of which the complex metal compounds are sparingly soluble to insoluble in water and in dilute alkalies, and treating the dyeings with agents yielding metal, wherein at least once in the course of the dyeing process the vegetable fibers are treated in a caustic alkaline medium at a raised temperature not exceeding the boiling point of the said medium.

5. Process for the production of fast tints on vegetable fibers, comprising dyeing the fibers with complex metal compounds of direct cotton dyestuffs in a caustic alkaline medium at a raised temperature not exceeding the boiling point of the said medium, the said complex metal compounds being sparingly soluble to insoluble in water and in dilute alkalies.

6. Process for the production of fast tints on vegetable fibers, comprising dyeing the fibers with complex metal compounds of direct cotton dyestuffs in a caustic alkaline medium containing compounds selected from the group consisting of ammonia and organic derivatives of ammonia, at a raised temperature not exceeding the boiling point of the said medium, the said complex metal compounds being sparingly soluble to insoluble in water and in dilute alkalies.

7. Process for the production of fast tints on vegetable fibers, comprising dyeing the fibers with direct cotton dyestuffs containing lake-forming groups, of which the complex copper compounds are sparingly soluble to insoluble in water and in dilute alkalies, and treating the dyeings with agents yielding copper stable towards dilute alkalies, wherein at least once in the course of the dyeing process the vegetable fibers are treated in a caustic alkaline medium at a raised temperature not exceeding the boiling point of said medium.

8. Process for the production of fast tints on vegetable fibers, comprising dyeing the fibers with complex copper compounds of direct cotton dyestuffs in a caustic alkaline medium at a raised temperature not exceeding the boiling point of the said medium, the said complex metal compounds being sparingly soluble to insoluble in water and in dilute alkalies.

FRITZ STRAUB.

WALTER HANHART.

WALTER ANDERAU. 70